# EUROPEAN PATENT SPECIFICATION

(11) **EP 2 937 449 B1**
(45) Date of publication and mention of the grant of the patent: **12.07.2017**
(21) Application number: 12891307.6
(22) Date of filing: 24.12.2012
(51) Int. Cl.: C25B 11/08, C25B 11/03, C25B 1/46

(54) **GAS DIFFUSION ELECTRODE AND PREPARATION METHOD THEREOF**
GASDIFFUSIONSELEKTRODE UND HERSTELLUNGSVERFAHREN DAFÜR
ÉLECTRODE DE DIFFUSION DE GAZ ET PROCÉDÉ DE PRÉPARATION CORRESPONDANT

(43) Date of publication of application: 28.10.2015
(73) Proprietor: Beijing University Of Chemical Technology, Beijing 100029 (CN)
(72) Inventor: WANG, Feng, Beijing 100029 (CN); CAO, Yinliang, Beijing 100029 (CN); LIU, Jingjun, Beijing 100029 (CN); LI, Zhilin, Beijing 100029 (CN)
(74) Representative: Lloyd, Patrick Alexander Desmond
(86) International application number: PCT/CN2012/001722
(87) International publication number: WO 2014/100912

(56) References cited:
- EP-A1- 0 014 896
- CN-A- 101 736 360
- CN-A- 101 774 666
- CN-A- 102 517 602
- US-A- 5 584 976
- US-B1- 6 399 236
- US-B1- 6 423 194

## Description

### Technical Field

The present invention relates to the field of chemical engineering, particularly to a gas diffusion electrode suitable for the chlor-alkali industry and a preparation method thereof.

### Background

As a basic chemical industry, chlor-alkali industry plays an important role in promoting national economic development. Meanwhile, chlor-alkali industry is an industry with high energy consumption, so how to reduce the energy consumption of chlor-alkali industry to a minimum has always been an issue focused by many countries.

Recently, the ion-exchange membrane brine electrolytic process with an oxygen diffusion cathode (substituting for a hydrogen evolution cathode), the nature of which is a hydrogen evolution reaction is replaced by an oxygen reduction reaction, receives more attention increasingly. The reaction equations of the traditional ion-exchange membrane brine electrolytic process with a hydrogen evolution electrode as the cathode are as follows:

2Cl⁻→Cl₂+2e (1.36V)

2H₂O+2e→2OH⁻+H₂ (-0.83V)

2NaCl+2H₂O→Cl₂+2NaOH+H₂ (2.19V),

In contrast, the electrochemical reaction equations of the ion-exchange membrane brine electrolytic process with an oxygen diffusion electrode as the cathode are as follows:

2Cl⁻→Cl₂+2e (1.36V)

O₂+2H₂O+4e→4OH⁻ (0.4V)

2NaCl+H₂O+1/2O₂→ Cl₂+2NaOH (0.96V).

It can be seen that, as for the ion-exchange membrane brine electrolytic process with an oxygen diffusion cathode substituting for a hydrogen evolution cathode, the theoretic decomposition voltage thereof can be reduced by 1.23 V, the theoretic energy thereof can be saved up to 40%, and the electric energy saved will be 700KWh per ton of alkali, which make the process have very considerable application value.

However, the original gas diffusion electrode begins in the development of fuel cell and zinc-air battery, which is relatively less applied to the chlor-alkali industry mainly because of the following aspects of difficulties:
1) the practical conditions of the electrolysis in chlor-alkali industry are relatively critical, usually under an alkali concentration of 30% or more and a temperature of 80-90°C, thus demanding relatively high requirement to the material and the preparation of the electrode;
2) during the electrochemical reaction of the oxygen diffusion cathode, influenced by the electro-catalysis mechanism of catalysts, two-electron side reaction will occur in some degree and produce a certain amount of HO₂⁻, which is corrosive to carbon material and thus bring negative effects to the structure, lifetime and electrochemical properties of the electrode;
3) the electrochemical reaction of the oxygen diffusion cathode is actually a process of gas-liquid-solid multiphase catalytic reaction, the balance of which is difficult to control, thus affecting the catalytic efficiency of the oxygen diffusion cathode;
4) the oxygen diffusion cathode cannot satisfy the requirements of large-scale industrial production for its low mechanical strength and high difficulty of installation; and
5) for the oxygen diffusion cathode, it is difficult to obtain an electrode having good surface condition without cracks, because the processes of dispersion and film formation of its slurry are complex and the requirement of its drying is high.

At present, to solve the aforesaid problems, a lot of research has been carried out in each country. For example, Japanese Patent Publication 2007-327092 discloses a gas diffusion electrode having high resistance of water-pressure but low speed of deterioration, which is prepared using AB-6 carbon black as hydrophobic carbon black, AB-12 carbon black as hydrophilic carbon black, and Ag powder as a catalyst. Japanese Patent Publication 2004-300451 discloses a gas diffusion electrode having stable performance, which is prepared with AB-6 carbon black as hydrophobic carbon black and Ag-plated metal web as a catalyst layer through the steps of dispersing the hydrophobic carbon black and an adhesive, filtering and drying, followed by hot-press molding the Ag-plated metal web, however such electrode is difficult to satisfy the requirement of large-scale industrial production of large electrode. Chinese Patent CN101736360A discloses a gas diffusion electrode having a structure that a Ni web plated with Ag as a support is disposed between a gas diffusion layer and a catalyst layer, however such electrode involves problems such as low mechanical strength, being liable to form cracks on the surface of the electrode during the production thereof and difficult to release during the hot pressing process, and thus cannot satisfy the requirement of industrial production.

### Summary

An object of the present invention is to provide a gas diffusion electrode which is simple and efficient as well as suitable for chlor-alkali industry, and a preparation method thereof so as to overcome the defects existed in prior art. Such object was achieved by the following technical solutions. In one aspect, the present invention relates to a gas diffusion electrode comprising a current collector, a gas diffusion layer, a gas catalysis layer coated on the gas diffusion layer, and a liquid guide layer located on the gas catalysis layer; wherein the gas diffusion layer comprises highly-graphitized carbon black and polytetrafluoroethylene (PTFE), and the gas catalysis layer comprises a catalyst, acidified highly-graphitized carbon black and polytetrafluoroethylene; the highly-graphitized carbon black is the carbon black having a peak intensity ratio I_{D}/I_{G} between 0.3 and 1.0 in the Raman spectrum, and the degrees of graphitization in the gas diffusion layer and the gas catalysis layer may be the same or different; the current collector and the liquid guide layer are both silver-plated metal foam having a thickness of 0.1-20 µm, and the silver-plated metal foam thereof may be the same or different.

In a preferred embodiment of the present invention, the mass ratio of the highly-graphitized carbon black to polytetrafluoroethylene in the gas diffusion layer is (0.01-1): (0.01-0.1).

In a preferred embodiment of the present invention, the mass ratio of the catalyst, the acidified highly-graphitized carbon black and polytetrafluoroethylene in the gas catalysis layer is (0.1-1): (0.1-1): (0.1-1).

In a preferred embodiment of the present invention, the metal of the silver-plated metal foam is selected from nickel, titanium, tungsten, cobalt, or alloys thereof.

In a preferred embodiment of the present invention, the catalyst in the gas catalysis layer is selected from silver powder or Ag/C composite catalyst; preferably, the catalyst has a particle size between 0.01 and 5 µm.

In a preferred embodiment of the present invention, the diffusion electrode is applied as a gas diffusion electrode in chlor-alkali industry.

In a preferred embodiment of the present invention, during the preparation of the gas diffusion electrode, the gas diffusion layer is prepared from raw materials comprising highly-graphitized carbon black, water, Triton, polytetrafluoroethylene emulsion and isopropanol in a mass ratio of (0.01-1): (0.1-1): (0.01-0.1): (0.01-0.1): 1, wherein the aqueous isopropanol solution of Triton is used as a dispersion medium.

In a preferred embodiment of the present invention, during the preparation of the gas diffusion electrode, the gas catalysis layer is prepared from raw materials comprising a catalyst, acidified highly-graphitized carbon black, water, Triton, polytetrafluoroethylene solution and isopropanol in a mass ratio of (0.1-1): (0.1-1): (1-10): (0.1-1): (0.1-1) : 1, wherein the aqueous solution of Triton is used as a dispersion medium.

In a preferred embodiment of the preparation method of the gas diffusion electrode according to the present invention, the preparation method of the gas diffusion layer comprises the following steps: (1) dispersing the highly-graphitized carbon black in the aqueous isopropanol solution comprising surfactant Triton, so as to obtain the slurry of the gas diffusion layer; dispersing this slurry by ultrasonic shear for 10 to 200 min; then adding 40 to 80 mass% of polytetrafluoroethylene emulsion, further dispersing by shear for 10 to 150 min; controlling the temperature during the dispersion of the gas diffusion layer slurry between 10 and 100°C, and the powder in the gas diffusion layer slurry having an average particle size between 0.2 and 10 µm after dispersion; setting the gas diffusion layer slurry for 5 to 100 h after dispersion; and controlling the solid content of the gas diffusion layer slurry between 5 and 40 wt%; and (2) coating the gas diffusion layer slurry evenly on the silver-plated metal foam of the current collector; after coating of the gas diffusion layer slurry, drying it at 40 to 120°C for 5-10 h; after coating and drying of the gas diffusion layer slurry, performing a primary cold-press molding treatment with a pressure between 0.1 and 2 MPa at a temperature between -10 and 50°C for a holding time between 10 and 300 s, so as to obtain an assembly of the current collector 1 and the gas diffusion layer 2.

In a preferred embodiment of the preparation method of the gas diffusion electrode according to the present invention, the preparation method of the gas catalysis layer comprises the following steps: (1) dispersing the catalyst, the acidified graphitized carbon black in the aqueous isopropanol solution comprising surfactant Triton, so as to obtain the catalysis layer slurry; dispersing this slurry by ultrasonic shear for 10-200 min; then adding 40-80 mass% of polytetrafluoroethylene emulsion, further dispersing by shear for 10-150 min; and controlling the temperature during the dispersion of the catalysis layer slurry between 10-100°C and the powder in the catalysis layer slurry having an average particle size between 0.2-10 µm after dispersion; and (2) coating the catalysis layer slurry evenly on the gas diffusion layer of the assembly of the gas diffusion layer and the current collector; drying it at 40-120°C for 0.5-1 h after coating of the catalysis layer slurry; after the coating and drying of the catalysis layer slurry, performing a secondary cold-press molding treatment to the assembly under a pressure between 0.1 and 2 MPa at a temperature between -10 and 50°C for a holding time between 10 and 300 s, so as to obtain a pre-molded gas diffusion electrode; baking the pre-molded gas diffusion electrode at high temperature between 270 and 290°C for 1 to 20 h; disposing the silver-plated metal foam of the liquid guide layer on the pre-molded gas diffusion electrode after baking, and performing hot-press molding thereto under a pressure between 2 and 12 MPa at a hot-press temperature between 330 and 450°C for a holding time between 10 and 300 s, thereby obtaining the gas diffusion electrode.

In a preferred embodiment of the above preparation method of the gas diffusion electrode, the silver-plated metal foam is prepared by plating Ag on the metal foam using electroplating, chemical plating, and replacement plating methods.

The catalyst used in the present invention includes Ag powder and Ag/C composite catalyst (the preparation thereof please refer to CN 101745390A), and the Ag/C composite catalysts mentioned in the context are all those prepared according to patent publication CN 101745390A.

The present invention has the following advantageous effects.

In the present invention, a gas diffusion layer, which has not only good electrical conductivity and gas permeability capability but also excellent resistance to water pressure, can be prepared by the processes of dispersing highly-graphitized carbon black in the aqueous isopropanol solution comprising a certain surfactant using ultrasonic shear and standing, so as to obtain a uniformly dispersed gas diffusion layer slurry; coating the gas diffusion layer slurry evenly on the silver-plated metal foam; and performing cold-pressing after drying the slurry. A pre-molded gas diffusion electrode can be prepared by dispersing the catalyst and the acidified highly-graphitized carbon black in the aqueous isopropanol solution comprising a certain surfactant using ultrasonic shear so as to obtain a uniformly dispersed catalysis layer slurry; coating the catalysis layer slurry evenly on the gas diffusion layer; and performing cold-pressing after drying the slurry. The catalysis layer obtained in this way not only has suitable hydrophilic and hydrophobic capacity which is beneficial to the gas-liquid-solid three-phase reaction, but also has anti-etching capacity and the capacity of preventing the occurrence of side reaction producing hydrogen peroxide, thus facilitating the long-term and stable operation of the electrode. The pre-molded gas diffusion electrode is subjected to high-temperature baking in order to thoroughly remove the residual surfactant in the interior of the electrode, thereby facilitating the uniform of the pore structure during the hot-press molding process. A gas diffusion electrode having a sandwich structure is formed by hot-pressing the silver-plated metal foam on the surface of the catalysis layer during the hot-pressing process, thus not only being beneficial to the progression of the three-phase reaction in the catalysis process, but also being capable of improving the electro-catalysis capacity of the electrode in a basic solution and the mechanical strength of the electrode itself due to the silver-plated metal foam. Therefore, the gas diffusion electrode provided by the present invention has good corrosion resistance and good electrical conductivity, and runs stably in a basic solution; thus it is suitable for the electrolysis reaction in chlor-alkali industry.

### Brief Description of the Drawings

Figure 1 is a schematic view showing the structure of the gas diffusion electrode provided by the present invention, wherein:
   1 - current collector, 2 - diffusion layer, 3 - catalysis layer, 4 - liquid guide layer;
Figure 2 is a Raman Spectrogram of the highly-graphitized carbon black in the gas diffusion layer provided by the present invention;
Figure 3 is the results of the rotating ring-disk test of the Ag powder catalyst in a basic solution; and
Figure 4 is the test data of the actual electrolysis of the gas diffusion electrodes prepared in Example 1 and Comparative Example 1. (Test conditions: in 30% NaOH solution, current density of 3KA/m²)

### Detailed Description of Certain Embodiments

### Example 1

The highly-graphitized carbon black used in this example is prepared by graphitizing carbon black (Vulcan XC-72) in a high-temperature graphitization furnace at 2700°C for 6-10 h, and a Raman Spectrogram for measuring the graphitization degree thereof is shown in Figure 2 with I_{D}/I_{G} of 0.67. The silver-plated nickel foam is prepared by electroplating, wherein the nickel foam is commercially available from Heze Tianyu Technical Developing Lt. Corp. The acidified highly-graphitized carbon black is prepared by refluxing the graphitized carbon black in nitric acid solution (68 mass%) at 120°C for 6 to 10 h. Specifically,
1) weighing 0.4-2 g highly-graphitized carbon black and dispersing it in an aqueous isopropanol solution comprising 0.4-1 g Triton, wherein the amount of isopropanol is 40 mL and the amount of water is 10-25 mL; then dispersing thus-obtained slurry by ultrasonic shear for 60 min, followed by adding 1-2 g of PTFE emulsion (D-110, 60 mass%); continuing performing shear dispersion for 10 min, and then coating the gas diffusion layer slurry evenly on silver-plated nickel foam with a size of 90 mm×90 mm after dispersion completed, after drying it in an oven at 60°C for 30 min, performing the primary cold-press molding with a pressure of 0.1-2 MPa at room temperature for 60 s, so as to obtain the assembly of the current collector 1 and the gas diffusion layer 2;
2) dispersing 1-2 g Ag powder catalyst and 2-3 g acidified graphitized carbon black in 2.5-3 g/L aqueous isopropanol solution of Triton so as to make the oxygen-containing functional group on the surface of the acidified graphitized carbon black in a concentration of 0.5-2 mmol/g, wherein the amount of isopropanol is 3 mL, and the amount of water is 15-30 mL; dispersing the slurry by ultrasonic shear for 60 min and then adding 2.5-3 g 60 mass% of PTFE emulsion; further dispersing by ultrasonic shear for 10 min; after the dispersion completed, coating the catalysis layer slurry on the gas diffusion layer of the assembly of the current collector 1 and the gas diffusion 2; after drying the slurry, performing the secondary cold-press molding treatment with a cold pressure of 0.1-2 MPa at room temperature for a holding time of 30 s, so as to obtain the pre-molded gas diffusion electrode, wherein the results of the rotating ring-disk test of the Ag powder catalyst in a basic solution are shown in Figure 3. It can be seen that the electro-catalysis mechanism is almost four-electron reaction;
3) baking the pre-molded gas diffusion electrode obtained by the above steps at high temperature which is controlled to 290°C for 2 h; and
4) disposing the silver-plated nickel foam of the guide layer on the pre-molded gas diffusion electrode subjected to baking, and performing hot-press molding to it with a pressure of 5-8 MPa at a hot-press temperature of 360°C for 60 s holding time, so as to obtain the gas diffusion electrode. The test data of the actual electrolysis of the gas diffusion electrode prepared is shown in Figure 4, which indicates that the gas diffusion electrode has good corrosion resistance and excellent and stable electrochemical performance in alkali solutions, and therefore, is suitable for electrolytic reactions in the chlorine alkali industry.

### Example 2

The highly-graphitized carbon black used in this example is prepared by graphitizing carbon black (Vulcan XC-72) at 2600°C for 2-15 h, and has a Raman Spectrogram with I_{D}/I_{G} of 0.7-1.0. The silver-plated nickel foam is prepared by electroplating, wherein the nickel foam is commercially available from Heze Tianyu Technical Developing Lt. Corp. The acidified highly-graphitized carbon black is prepared by refluxing the graphitized carbon black in nitric acid solution (68 mass%) at 140°C for 6 to 10 h. Specifically,
1) weighing 1-3 g highly-graphitized carbon black and dispersing it in an aqueous isopropanol solution comprising 0.4-3 g Triton, wherein the amount of isopropanol is 40 mL and the amount of water is 4-16 mL; then dispersing thus-obtained slurry by ultrasonic shear for 60 min, followed by adding 0.4-1.5 g of PTFE emulsion (D-110, 60 mass%); continuing performing shear dispersion for 10 min, and then coating the gas diffusion layer slurry evenly on silver-plated nickel foam with a size of 90 mm×90 mm after dispersion completed; after drying it in an oven at 60°C for 30 min, performing the primary cold-press molding with a cold pressure of 0.1-2 MPa at room temperature for 60 s, so as to obtain the assembly of the current collector 1 and the gas diffusion layer 2;
2) dispersing 0.3-1.5 g Ag powder catalyst orAg/Carbon composite catalyst and 0.5-2 g acidified graphitized carbon black in 0.3-1.8 g/L aqueous isopropanol solution of Triton so as to make the oxygen-containing functional group on the surface of the acidified graphitized carbon black in a concentration of 1.5-4 mmol/g, wherein the amount of isopropanol is 3 mL, and the amount of water is 3-8 mL; dispersing the slurry by ultrasonic shear for 60 min and then adding 0.3-1.5 g of PTFE emulsion (60 mass%); further dispersing by ultrasonic shear for 10 min; after the dispersion completed, coating the catalysis layer slurry on the gas diffusion layer of the assembly of the current collector 1 and the gas diffusion 2; after drying the slurry, performing the secondary cold-press molding treatment with a cold pressure of 0.1-2 MPa at room temperature for a holding time of 30 s, so as to obtain the pre-molded gas diffusion electrode;
3) baking the pre-molded gas diffusion electrode obtained by the above steps at high temperature which is controlled to 280°C for 4 h; and
4) disposing the silver-plated nickel foam of the guide layer on the pre-molded gas diffusion electrode subjected to baking, and performing hot-press molding to it with a pressure of 2-5 MPa at a hot-press temperature of 370°C for a holding time of 180 s, so as to obtain the gas diffusion electrode.

### Example 3

The highly-graphitized carbon black used in this example is prepared by graphitizing carbon black (Vulcan XC-72) in a high-temperature graphitization furnace at 2900°C for 2-15 h, and has a Raman Spectrogram with I_{D}/I_{G} of 0.3-0.6. The silver-plated nickel foam is prepared by electroplating, wherein the nickel foam is commercially available from Heze Tianyu Technical Developing Lt. Corp. The acidified highly-graphitized carbon black is prepared by refluxing the graphitized carbon black in nitric acid solution (68 mass%) at 160°C for 6 to 10 h. Specifically,
1) weighing 2-4 g highly-graphitized carbon black and dispersing it in an aqueous isopropanol solution comprising 2.5-4 g Triton, wherein the amount of isopropanol is 40 mL and the amount of water is 20-40 mL; then dispersing thus-obtained slurry by ultrasonic shear for 60 min, followed by adding 1.8-4 g of PTFE emulsion (D-110, 60 mass%); continuing performing shear dispersion for 10 min, and then coating the gas diffusion layer slurry evenly on silver-plated nickel foam with a size of 90 mm×90 mm after dispersion completed; after drying it at 60°C for 30 min, performing the primary cold-press molding in a cold press machine with a cold pressure of 1.5-2 MPa at room temperature for 60 s, so as to obtain the assembly of the current collector 1 and the gas diffusion layer 2;
2) dispersing 2-3 g Ag powder catalyst or Ag/Carbon composite catalyst and 0.3-1 g acidified graphitized carbon black in 1.5-2.8 g/L aqueous isopropanol solution of Triton so as to make the oxygen-containing functional group on the surface of the acidified graphitized carbon black in a concentration of 3.5-5 mmol/g, wherein the amount of isopropanol is 3 mL, and the amount of water is 5-15mL; dispersing the slurry by ultrasonic shear for 60 min and then adding 1.4-2.8 g of PTFE emulsion (60 mass%); further dispersing by ultrasonic shear for 10 min; after the dispersion completed, coating the catalysis layer slurry on the gas diffusion layer of the assembly of the current collector 1 and the gas diffusion 2; after drying the slurry, performing the secondary cold-press molding treatment with a cold pressure of 1.5-2 MPa at room temperature for a holding time of 30 s, so as to obtain the pre-molded gas diffusion electrode;
3) baking the pre-molded gas diffusion electrode obtained by the above steps at high temperature which is controlled to 270°C for 6 h; and
4) disposing the silver-plated nickel foam of the guide layer on the pre-molded gas diffusion electrode subjected to baking, and performing hot-press molding to it with a pressure of 8-12 MPa at a hot-press temperature of 350°C for a holding time of 30 s, so as to obtain the gas diffusion electrode.

### Comparative Example 1

The highly-graphitized carbon black used herein is prepared by graphitizing carbon black (Vulcan XC-72) in a high-temperature graphitization furnace at 2700°C for 6-10 h, and a Raman Spectrogram for measuring the graphitization degree thereof is shown in Figure 2 with I_{D}/I_{G} of 0.67. The silver-plated nickel foam is prepared by electroplating, wherein the nickel foam is commercially available from Heze Tianyu Technical Developing Lt. Corp. The acidified highly-graphitized carbon black is prepared by refluxing the graphitized carbon black in nitric acid solution (68 mass%) at 120°C for 6 to 10 h. Specifically,
1) weighing 0.4-2 g highly-graphitized carbon black and dispersing it in an aqueous isopropanol solution comprising 0.4-1 g Triton, wherein the amount of isopropanol is 40 mL and the amount of water is 10-25 mL; then dispersing thus-obtained slurry by ultrasonic shear for 60 min, followed by adding 1-2 g of PTFE emulsion (D-110, 60 mass%); continuing performing shear dispersion for 10 min, and then coating the gas diffusion layer slurry evenly on silver-plated nickel foam with a size of 90 mm×90 mm after dispersion completed, after drying it in an oven at 60°C for 30 min, performing the primary cold-press molding with a cold pressure of 0.1-2 MPa at room temperature for 60 s, so as to obtain the assembly of the current collector 1 and the gas diffusion layer 2;
2) dispersing 1-2 g Ag powder catalyst and 2-3 g acidified graphitized carbon black in 2.5-3 g/L aqueous isopropanol solution of Triton so as to make the oxygen-containing functional group on the surface of the acidified graphitized carbon black in a concentration of 0.5-2 mmol/g, wherein the amount of isopropanol is 3 mL, and the amount of water is 15-30 mL; dispersing the slurry by ultrasonic shear for 60 min and then adding 2.5-3 g 60 mass% of PTFE emulsion; further dispersing by ultrasonic shear for 10 min; after the dispersion completed, coating the catalysis layer slurry on the gas diffusion layer of the assembly of the current collector 1 and the gas diffusion 2; after drying the slurry, performing the secondary cold-press molding treatment with a cold pressure of 0.1-2 MPa at room temperature for a holding time of 30 s, so as to obtain the pre-molded gas diffusion electrode;
3) baking the pre-molded gas diffusion electrode obtained by the above steps at high temperature which is controlled to 290°C for 2 h; and
4) disposing the pre-molded gas diffusion electrode after baking directly on a hot press machine and performing hot-press molding to it with a hot pressure of 5-8 MPa at a hot-press temperature of 360°C for a holding time of 60 s, so as to obtain the gas diffusion electrode. The test data of the actual electrolysis of the gas diffusion electrode prepared is shown in Figure 4, which indicates that the electrolysis properties thereof show degradation in a basic solution with the elapse of time, thus the electrode is not suitable for the long-term electrolysis reaction in chlor-alkali industry.

It should be understood that, for a person skilled in the art, the embodiments would be modified or varied in accordance with the above description, and all such modifications and variations are within the scope of the invention as specifically set forth in the claims appended hereto.

## Claims

1. A gas diffusion electrode comprising a current collector, a gas diffusion layer, a gas catalysis layer coated on the gas diffusion layer, and a liquid guide layer located on the gas catalysis layer; wherein the gas diffusion layer comprises highly-graphitized carbon black and polytetrafluoroethylene, and the gas catalysis layer comprises a catalyst, acidified highly-graphitized carbon black and polytetrafluoroethylene; the highly-graphitized carbon black is the carbon black having a peak intensity ratio I_{D}/I_{G} between 0.3 and 1.0 in the Raman spectrum, and preferably the concentration of the oxygen-containing functional group on the surface of the acidified graphitized carbon black is 0.5-2 mmol/g; the degrees of graphitization in the gas diffusion layer and the gas catalysis layer may be the same or different; the current collector and the liquid guide layer are both silver-plated metal foam having a thickness of 0.1-20 µm, and the silver-plated metal foam thereof may be the same or different.

2. The gas diffusion electrode according to claim 1, wherein the mass ratio of the highly-graphitized carbon black to polytetrafluoroethylene in the gas diffusion layer is (0.01-1): (0.01-0.1).

3. The gas diffusion electrode according to claim 1, wherein the mass ratio of the catalyst, the acidified highly-graphitized carbon black and polytetrafluoroethylene in the gas catalysis layer is (0.1-1): (0.1-1): (0.1-1).

4. The gas diffusion electrode according to any one of claims 1-3, wherein the metal of the silver-plated metal foam is selected from nickel, titanium, tungsten, cobalt, or alloys thereof.

5. The gas diffusion electrode according to claim 1, wherein the catalyst in the gas catalysis layer is selected from silver powder or Ag/C composite catalyst; preferably, the catalyst has a particle size between 0.01 and 5 µm.

6. The gas diffusion electrode according to any one of claims 1-5, wherein the diffusion electrode is a gas diffusion electrode applied in chlor-alkali industry.

7. A method for preparing the gas diffusion electrode according to claim 6, wherein the gas diffusion layer is prepared from raw materials comprising highly-graphitized carbon black, water, Triton, polytetrafluoroethylene emulsion and isopropanol in a mass ratio of (0.01-1) : (0.1-1) : (0.01-0.1) : (0.01-0.1) : 1, wherein the aqueous isopropanol solution of Triton is used as a dispersion medium.

8. A method for preparing the gas diffusion electrode according to claim 6, wherein the gas catalysis layer is prepared from raw materials comprising a catalyst, acidified highly-graphitized carbon black, water, Triton, polytetrafluoroethylene solution and isopropanol in a mass ratio of (0.1-1) : (0.1-1) : (1-10) : (0.1-1) : (0.1-1) : 1, wherein the aqueous isopropanol solution of Triton is used as a dispersion medium.

9. The method for preparing the gas diffusion electrode according to claim 7, wherein the preparation method of the gas diffusion layer comprises the following steps:
(1) dispersing the highly-graphitized carbon black in the aqueous isopropanol solution comprising surfactant Triton, so as to obtain a slurry of the gas diffusion layer; dispersing this slurry by ultrasonic shear for 10 to 200 min; then adding 40 to 80 mass% of polytetrafluoroethylene emulsion, further dispersing by shear for 10 to 150 min; controlling the temperature during the dispersion of the gas diffusion layer slurry between 10 and 100°C and after dispersion the powder in the gas diffusion layer slurry having an average particle size between 0.2 and 10 µm; setting the gas diffusion layer slurry for 5 to 100 h after dispersion; and controlling the solid content of the gas diffusion layer slurry between 5 and 40 wt%; and
(2) coating the gas diffusion layer slurry evenly on the silver-plated metal foam of the current collector; after coating of the gas diffusion layer slurry, drying it at 40 to 120°C for 5-10 h; after coating and drying of the gas diffusion layer slurry, performing a primary cold-press molding treatment at a cold pressure between 0.1 and 2 MPa, a temperature between -10 and 50°C and a holding time between 10 and 300 s, so as to obtain an assembly of the current collector and the gas diffusion layer.

10. The method for preparing the gas diffusion electrode according to claim 8, wherein the preparation method of the gas catalysis layer comprises the following steps:
(1) dispersing the catalyst, the acidified graphitized carbon black in the aqueous isopropanol solution comprising surfactant Triton, so as to obtain a catalysis layer slurry; dispersing this slurry by ultrasonic shear for 10-200 min; then adding 40-80 mass% of polytetrafluoroethylene emulsion, further dispersing by shear for 10-150 min; and controlling the temperature during the dispersion of the catalysis layer slurry between 10-100°C and the powder in the catalysis layer slurry having an average particle size between 0.2-10 µm after dispersion; and
(2) coating the catalysis layer slurry evenly on the gas diffusion layer of the assembly of the gas diffusion layer and the current collector; drying it at 40-120°C for 0.5-1 h after coating of the catalysis layer slurry; after the coating and drying of the catalysis layer slurry, performing a secondary cold-press molding treatment to the assembly under a cold pressure between 0.1 and 2 MPa at a temperature between -10 and 50°C for a holding time between 10 and 300 s, so as to obtain a pre-molded gas diffusion electrode; baking the pre-molded gas diffusion electrode at high temperature between 270 and 290°C for 1 to 20 h; disposing the silver-plated metal foam of the liquid guide layer on the pre-molded gas diffusion electrode after baking, and performing hot-press molding thereto under a hot pressure between 2 and 12 MPa at a hot-press temperature between 330 and 450°C for a holding time between 10 and 300 s, thereby obtaining the gas diffusion electrode.

## Patentansprüche

1. Gasdiffusionselektrode, umfassend einen Stromabnehmer, eine Gasdiffusionsschicht, eine auf der Gasdiffusionsschicht beschichtete Gaskatalyseschicht und eine auf der Gaskatalyseschicht befindliche flüssige Führungsschicht; wobei die Gasdiffusionsschicht hoch graphitierten Ruß und Polytetrafluorethylen umfasst und die Gaskatalyseschicht einen Katalysator, angesäuerten hoch graphitierten Ruß und Polytetrafluorethylen umfasst; der hoch graphitierte Ruß der Ruß mit einem Peak-Intensitätsverhältnis I_{D}/I_{G} zwischen 0,3 und 1,0 im Raman-Spektrum ist, und vorzugsweise wobei die Konzentration der sauerstoffhaltigen Funktionsgruppe auf der Oberfläche des angesäuerten graphitierten Rußes 0,5-2 mmol/g beträgt; die Graphitisierungsgrade in der Gasdiffusionsschicht und der Gaskatalyseschicht gleich oder verschieden sein können; der Stromabnehmer und die flüssige Führungsschicht beide versilberter Metallschaum mit einer Dicke von 0,1-20 µm sind und der versilberte Metallschaum davon gleich oder verschieden sein kann.

2. Gasdiffusionselektrode nach Anspruch 1, wobei das Massenverhältnis des hoch graphitierten Rußes zu Polytetrafluorethylen in der Gasdiffusionsschicht (0,01-1) : (0,01-0,1) beträgt.

3. Gasdiffusionselektrode nach Anspruch 1, wobei das Massenverhältnis des Katalysators, des angesäuerten hoch graphitierten Rußes und des Polytetrafluorethylens in der Gaskatalyseschicht (0,1-1): (0,1-1): (0,1-1) beträgt.

4. Gasdiffusionselektrode nach einem der Ansprüche 1-3, wobei das Metall des versilberten Metallschaums ausgewählt ist aus Nickel, Titan, Wolfram, Cobalt und Legierungen davon.

5. Gasdiffusionselektrode nach Anspruch 1, wobei der Katalysator in der Gaskatalyseschicht ausgewählt ist aus Silberpulver und Ag/C-Verbundkatalysator; vorzugsweise wobei der Katalysator eine Partikelgröße zwischen 0,01 und 5 µm aufweist.

6. Gasdiffusionselektrode nach einem der Ansprüche 1-5, wobei die Diffusionselektrode eine in der Chlor-Alkali-Industrie angewandte Gasdiffusionselektrode ist.

7. Verfahren zum Herstellen der Gasdiffusionselektrode nach Anspruch 6, wobei die Gasdiffusionsschicht aus Rohstoffen hergestellt wird, die Folgendes umfassen: hoch graphitierten Ruß, Wasser, Triton, Polytetrafluorethylenemulsion und Isopropanol in einem Massenverhältnis von (0,01-1): (0,1-1): (0,01-0.1): (0,01-0.1): 1, wobei die wässrige Isopropanollösung aus Triton als ein Dispersionsmittel verwendet wird.

8. Verfahren zum Herstellen der Gasdiffusionselektrode nach Anspruch 6, wobei die Gaskatalyseschicht aus Rohstoffen hergestellt wird, die Folgendes umfassen: einen Katalysator, angesäuerten hoch graphitierten Ruß, Wasser, Triton, Polytetrafluorethylenlösung und Isopropanol in einem Massenverhältnis von (0,1-1) : (0,1-1) : (1-10) : (0,1-1): (0,1-1) : 1, wobei die wässrige Isopropanollösung aus Triton als ein Dispersionsmittel verwendet wird.

9. Verfahren zum Herstellen der Gasdiffusionselektrode nach Anspruch 7, wobei das Herstellungsverfahren der Gasdiffusionsschicht die folgenden Schritte umfasst:
(1) Dispergieren des hoch graphitierten Rußes in der wässrigen Isopropanollösung, umfassend Tensid Triton, um eine Aufschlämmung der Gasdiffusionsschicht zu erhalten; Dispergieren dieser Aufschlämmung durch Ultraschallscherung 10 bis 200 min lang; dann Hinzugeben von 40 bis 80 Ma.-% Polytetrafluorethylenemulsion, ferner Dispergieren durch Scherung 10 bis 150 min lang; Regeln der Temperatur während des Dispergierens der Gasdiffusionsschichtaufschlämmung zwischen 10 und 100 °C und wobei nach dem Dispergieren das Pulver in der Gasdiffusionsschichtaufschlämmung eine durchschnittliche Partikelgröße zwischen 0,2 und 10 µm aufweist; Einstellen der Gasdiffusionsschichtaufschlämmung 5 bis 100 h nach dem Dispergieren; und Steuern des Feststoffgehalts der Gasdiffusionsschichtaufschlämmung zwischen 5 und 40 Gew.-%; und
(2) Beschichten der Gasdiffusionsschichtaufschlämmung gleichmäßig auf dem versilberten Metallschaum des Stromabnehmers; nach dem Beschichten der Gasdiffusionsschichtaufschlämmung, Trocknen dieser bei 40 bis 120 °C 5-10 h lang; nach dem Beschichten und Trocknen der Gasdiffusionsschichtaufschlämmung, Durchführen einer primären Kaltpressformbehandlung bei einem kalten Druck zwischen 0,1 und 2 MPa, einer Temperatur zwischen -10 und 50 °C und einer Verweilzeit zwischen 10 und 300 s, um eine Anordnung des Stromabnehmers und der Gasdiffusionsschicht zu erhalten.

10. Verfahren zum Herstellen der Gasdiffusionselektrode nach Anspruch 8, wobei das Herstellungsverfahren der Gaskatalyseschicht die folgenden Schritte umfasst:
(1) Dispergieren des Katalysators, des angesäuerten graphitierten Rußes in der wässrigen Isopropanollösung, umfassend Tensid Triton, um eine Katalyseschichtaufschlämmung zu erhalten; Dispergieren dieser Aufschlämmung durch Ultraschallscherung 10 bis 200 min lang; dann Hinzugeben von 40 bis 80 Ma.-% Polytetrafluorethylenemulsion, ferner Dispergieren durch Scherung 10-150 min lang; und Regeln der Temperatur während des Dispergierens der Katalyseschichtaufschlämmung auf 10-100 °C und wobei das Pulver in der Katalyseschichtaufschlämmung nach dem Dispergieren eine durchschnittliche Partikelgröße von 0,2-10 µm aufweist; und
(2) Beschichten der Katalyseschichtaufschlämmung gleichmäßig auf der Gasdiffusionsschicht der Anordnung der Gasdiffusionsschicht und des Stromabnehmers; Trocknen bei 40-120 °C 0,5-1 h lang nach dem Beschichten der Katalyseschichtaufschlämmung; nach dem Beschichten und Trocknen der Katalyseschichtaufschlämmung, Durchführen einer sekundären Kaltpressformbehandlung der Anordnung bei einem kalten Druck zwischen 0,1 und 2 MPa bei einer Temperatur zwischen -10 und 50 °C und einer Verweilzeit zwischen 10 und 300 s, um eine vorgeformte Gasdiffusionselektrode zu erhalten; Brennen der vorgeformten Gasdiffusionselektrode bei hoher Temperatur zwischen 270 und 290 °C 1 bis 20 h lang; Anordnen des versilberten Metallschaums der flüssigen Führungsschicht auf der vorgeformten Gasdiffusionselektrode nach dem Brennen, und Durchführen eines Warmpressformens davon bei einem heißen Druck zwischen 2 und 12 MPa bei einer Warmpresstemperatur zwischen 330 und 450 °C und einer Verweilzeit zwischen 10 und 300 s, dadurch Erhalten der Gasdiffusionselektrode.

## Revendications

1. Electrode à diffusion de gaz comprenant un collecteur de courant, une couche de diffusion de gaz, une couche de catalyse de gaz revêtue sur la couche de diffusion de gaz et une couche de guidage de liquide située sur la couche de catalyse de gaz ; dans laquelle la couche de diffusion de gaz comprend du noir de carbone hautement graphitisé et du polytétrafluoroéthylène, et la couche de catalyse de gaz comprend un catalyseur, du noir de carbone hautement graphitisé acidifié et du polytétrafluoroéthylène ; le noir de carbone hautement graphitisé est le noir de carbone ayant un rapport d'intensité de crête I_{D}/I_{G} entre 0,3 et 1,0 dans le spectre de Raman, et de préférence la concentration du groupe fonctionnel contenant de l'oxygène sur la surface du noir de carbone graphitisé acidifié est de 0,5 à 2 mmoles/g ; les degrés de graphitisation dans la couche de diffusion de gaz et la couche de catalyse de gaz peuvent être les mêmes ou différents ; le collecteur de courant et la couche de guidage de liquide sont tous deux une mousse en métal plaquée argent ayant une épaisseur de 0,1 à 20 µm, et leur mousse en métal plaquée argent peut être la même ou différente.

2. Electrode à diffusion de gaz selon la revendication 1, dans laquelle le rapport en masse entre le noir de carbone hautement graphitisé et le polytétrafluoroéthylène dans la couche de diffusion de gaz est (0,01 à 1) : (0,01 à 0,1).

3. Electrode à diffusion de gaz selon la revendication 1, dans laquelle le rapport en masse entre le catalyseur, le noir de carbone hautement graphitisé acidifié et le polytétrafluoroéthylène dans la couche de catalyse de gaz est (0,1 à 1) : (0,1 à 1) : (0,1 à 1).

4. Electrode à diffusion de gaz selon l'une quelconque des revendications 1 à 3, dans laquelle le métal de la mousse en métal plaquée argent est choisi parmi le nickel, le titane, le tungstène, le cobalt ou leurs alliages.

5. Electrode à diffusion de gaz selon la revendication 1, dans laquelle le catalyseur dans la couche de catalyse de gaz est choisi parmi une poudre d'argent ou un catalyseur composite Ag/C ; de préférence, le catalyseur a une taille de particules entre 0,01 et 5 µm.

6. Electrode à diffusion de gaz selon l'une quelconque des revendications 1 à 5, dans laquelle l'électrode à diffusion est une électrode à diffusion de gaz appliquée dans l'industrie du chlore et de la soude.

7. Procédé de préparation de l'électrode à diffusion de gaz selon la revendication 6, dans lequel la couche de diffusion de gaz est préparée à partir de matières premières comprenant du noir de carbone hautement graphitisé, de l'eau, du Triton, une émulsion de polytétrafluoroéthylène et de l'isopropanol dans un rapport en masse de (0,01 à 1) : (0,1 à 1) : (0,01 à 0,1) : (0,01 à 0,1) : 1, dans lequel la solution d'isopropanol aqueuse de Triton est utilisée en tant que milieu de dispersion.

8. Procédé de préparation de l'électrode à diffusion de gaz selon la revendication 6, dans lequel la couche de catalyseur de gaz est préparée à partir de matières premières comprenant un catalyseur, du noir de carbone hautement graphitisé acidifié, de l'eau, du Triton, une solution de polytétrafluoroéthylène et de l'isopropanol dans un rapport en masse de (0,1 à 1) : (0,1 à 1) : (1 à 10) : (0,1 à 1) : (0,1 à 1) : 1, dans lequel la solution d'isopropanol aqueuse de Triton est utilisée comme milieu de dispersion.

9. Procédé de préparation de l'électrode à diffusion de gaz selon la revendication 7, dans lequel le procédé de préparation de la couche de diffusion de gaz comprend les étapes suivantes :
(1) dispersion du noir de carbone hautement graphitisé dans la solution d'isopropanol aqueuse comprenant du tensioactif Triton, de façon à obtenir une bouillie de la couche de diffusion de gaz ; dispersion de cette bouillie par cisaillement ultrasonique pendant 10 à 200 min ; puis ajout de 40 à 80 % en masse d'une émulsion de polytétrafluoroéthylène, dispersion en outre par cisaillement pendant 10 à 150 min ; régulation de la température pendant la dispersion de la bouillie de couche de diffusion de gaz entre 10 et 100 °C et après dispersion la poudre dans la bouillie de couche de diffusion de gaz ayant une taille de particules moyenne entre 0,2 et 10 µm ; durcissement de la bouillie de couche de diffusion de gaz pendant 5 à 100 h après dispersion ; et régulation de la teneur en matière solide de la bouillie de couche de diffusion de gaz entre 5 et 40 % en poids ; et
(2) revêtement de la bouillie de couche de diffusion de gaz de façon régulière sur la mousse en métal plaquée argent du collecteur de courant ; après revêtement de la bouillie de couche de diffusion de gaz, son séchage à 40 à 120 °C pendant 5 à 10 h ; après revêtement et séchage de la bouillie de couche de diffusion de gaz, réalisation d'un traitement de moulage à la presse à froid primaire à une pression à froid entre 0,1 et 2 MPa, une température entre -10 et 50 °C et un temps de maintien entre 10 et 300 s, de façon à obtenir un assemblage du collecteur de courant et de la couche de diffusion de gaz.

10. Procédé de préparation de l'électrode à diffusion de gaz selon la revendication 8, dans lequel le procédé de préparation de la couche de catalyse de gaz comprend les étapes suivantes :
(1) dispersion du catalyseur, du noir de carbone graphitisé acidifié dans la solution d'isopropanol aqueuse comprenant du tensioactif Triton, de façon à obtenir une bouillie de couche de catalyse ; dispersion de cette bouillie par cisaillement ultrasonique pendant 10 à 200 min ; puis ajout de 40 à 80 % en masse d'émulsion de polytétrafluoroéthylène, dispersion en outre par cisaillement pendant 10 à 150 min ; et régulation de la température pendant la dispersion de la bouillie de couche de catalyse entre 10 et 100 °C et la poudre dans la bouillie de couche de catalyse ayant une taille de particules moyenne entre 0,2 et 10 µm après dispersion ; et
(2) revêtement de la bouillie de couche de catalyse de façon régulière sur la couche de diffusion de gaz de l'assemblage de la couche de diffusion de gaz et du collecteur de courant ; son séchage à 40 à 120 °C pendant 0,5 à 1 h après revêtement de la bouillie de couche de catalyse ; après le revêtement et le séchage de la bouillie de couche de catalyse, réalisation d'un traitement de moulage à la presse à froid secondaire sur l'assemblage à une pression à froid entre 0,1 et 2 MPa à une température entre -10 et 50 °C pendant un temps de maintien entre 10 et 300 s, de façon à obtenir une électrode à diffusion de gaz pré-moulée ; cuisson de l'électrode à diffusion de gaz pré-moulée à une température élevée entre 270 et 290 °C pendant 1 à 20 h ; dépôt de la mousse en métal plaquée argent de la couche de guidage de liquide sur l'électrode à diffusion de gaz pré-moulée après cuisson, et réalisation d'un moulage à la presse à chaud sur celle-ci à une pression à chaud entre 2 et 12 MPa à une température de presse à chaud entre 330 et 450 °C pendant un temps de maintien entre 10 et 300 s, obtenant ainsi l'électrode à diffusion de gaz.
